

# UNITED STATES PATENT OFFICE.

WILLIAM RINTOUL, THOMAS JOSEPH NOLAN, AND OLIVER WARD STICKLAND, OF STEVENSTON, SCOTLAND, ASSIGNEES TO NOBEL'S EXPLOSIVES COMPANY, LIMITED, OF STEVENSTON, SCOTLAND.

## EXPLOSIVE.

1,392,851.

Specification of Letters Patent.

Patented Oct. 4, 1921.

No Drawing.

Application filed October 19, 1920. Serial No. 418,082.

To all whom it may concern:

Be it known that we, WILLIAM RINTOUL, THOMAS JOSEPH NOLAN, and OLIVER WARD STICKLAND, all subjects of the King of Great Britain and Ireland, and all residing at Ardeer Factory, Stevenston, Ayrshire, Scotland, have invented certain new and useful Improvements in Explosives, (for which we have filed an application in Great Britain October 10, 1919,) of which the following is a specification.

This invention relates to the manufacture or hardened granulated fibrous nitrocellulose powders for shot-guns consisting of mixtures of fibrous nitrocellulose, metallic nitrates and moderating ingredients that are granulated and subsequently hardened by treatment with a solvent medium that does not destroy the fibrous appearance of the grains. Examples of this class of explosives are the well known shotgun powders "Schultze" and "E. C."

It does not relate to gelatinized or colloided propellant powders, for example, such as are described in United States Patents Nos. 1,311,909 and 1,312,463 nor powders for military small arms and cannons.

The present process, apart from dealing only with grains which are not suitable for military propellant purposes differs from these patents by the essential use of a non-volatile gelatinizer for hardening, without which gelatinizing property and desired hardening effect cannot be obtained, although to produce the deterrent effect aimed at in the patents numbered as above, does not necessarily require the use of a gelatinizer.

This class of explosive has hitherto been manufactured broadly as follows:—Nitrocellulose of various degrees of solubility in a mixture of ether and alcohol, is mixed or incorporated with metallic nitrates with or without starch and other moderating ingredients such as mineral jelly or other well known moderators. The wet mechanical mixture is subdivided by being passed through a sieve and the rough particles so produced formed into grains by revolving in pans, or by shaking on vibrating plates or by other means. The dried grains are too soft for the purposes required, and it is the practice to harden them by moistening with volatile solvents that have a solvent action

on the nitrocellulose base, thereby on drying 55 hardening the grains. The solvents that are in use or have been used consist of mixtures of ether and alcohol, camphor and alcohol, volatile solvents of nitrocellulose such as acetone, ethyl methyl ketone, amyl acetate, etc., 60 diluted by alcohol, benzene, petroleum ether or similar medium or mixture of these, and considerable quantities of these solvents are required for hardening.

It is well known that the method of hardening described above is an expensive operation even when solvent recovery is attempted, and the principal object of the invention is to improve or simplify the production of this class of explosive by eliminating or reducing the amount of volatile solvent required in the hardening operation.

Now we have discovered that useful hardened granulated fibrous nitrocellulose explosives can be manufactured by the employment of a non-volatile gelatinizing agent, 75 that is a gelatinizing agent of such a degree of freedom from volatility as to remain substantially in the powder. Thus we have found that by spraying a non-volatile solvent, (which may or may not be miscible with water but is preferably not so miscible) 80 on to the wet grains and then drying out the water say by a stoving operation, only one such operation need be employed instead of 85 two as are required according to common practice.

The invention consists in hardened granulated fibrous nitrocellulose explosives in which the hardening has been effected by the 90 aid of non-volatile gelatinizing agents, and in processes for producing such powders.

The invention further consists in incorporating a non-volatile gelatinizing agent in the manufacture of the grains and in bringing about hardening of the grains thereby.

The invention also consists in treating the grains with a liquid non-volatile gelatinizer, preferably in a finely divided state as in a spray, whereby hardening of the grains is 100 effected.

The invention further consists in treating the grains with a solid non-volatile gelatinizer in a finely divided state whereby hardening of the grains is effected.

The invention also consists in treating the grains with an aqueous solution of a non-volatile gelatinizer preferably in a finely di-

vided state as in a spray whereby hardening of the grains is effected.

The invention further consists in treating the grains with a practically concentrated 5 solution of a non-volatile gelatinizer in a volatile organic medium.

In carrying the invention into effect in one form we bring about the hardening of the grain by the combined gelatinizing 10 effect of a reduced quantity of volatile solvent and that of an added non-volatile gelatinizing agent such as:—

- (1) Urethanes or esters of substituted carbaminic acid.
- 15 (2) Anilids or their homologues.
- (3) Substituted ureas.
- (4) Condensation products of glycerol and other polyhydric alcohols with aldehydes.
- (5) Homologues of oxanilic ester.
- 20 (6) Non-volatile esters of organic acids or mixtures thereof. Examples of some of these gelatinizers applied to another purpose utilizing the combined gelatinizing effect with nitroglycerin are published in British 25 patent specifications Nos. 4940 and 4941 of 1913. The wet mixture of nitrocellulose, metallic nitrates moderating ingredients and non-volatile gelatinizing agent is granulated in any well known manner and dried. The 30 dried grains are then moistened in any convenient manner with a volatile medium having little or no hardening effect in the absence of a non-volatile gelatinizer in the explosive, such as, for example, a mixture of 35 alcohol and benzene. We have found that the percentage on the explosive grains of the volatile medium required to harden is substantially less than that necessary when these non-volatile gelatinizers are not ingredients of the explosive.

In order that the form of our invention may be more fully understood we will describe one example and method of production. A wet mixture of 76 parts of nitro- 45 cellulose, 10 parts of barium nitrate, 2 parts of potassium nitrate and 12 parts of a liquid mixture of formanilid and form-o-toluidid are mixed and incorporated under an edge runner. This mixture is rubbed through a 50 sieve 10 meshes to the inch and the sifted material placed in a steam heated revolving pan until the grains are correctly formed and contain about 50% of water. The correct sizes of grains are then sifted out and 55 dried. On to 100 parts by weight of the dried grains 10 parts by weight of a mixture of alcohol and benzene are added by means of a rose and the slightly moistened explosive grains placed in a closed vessel 60 for a few hours so that the volatile medium may uniformly spread throughout the mass. Subsequently the grains are dried and the hardening is effected.

In carrying the invention into effect in 65 another form in which the quantity of vola-

tile solvent is greatly reduced we harden granulated fibrous nitrocellulose explosives by spraying on to the dry or preferably wet grains a concentrated solution of a non-volatile gelatinizing agent in a volatile or 70 organic medium.

Thus we select the volatile organic medium having regard to the solubility of the particular gelatinizer therein and its suitability for the operation in view. We place 75 the wet or dry grains in a revolving vessel and while the grains are being moved about bring them into contact with the finely divided or atomized solution of the gelatinizer by means of any convenient atomizing 80 or spraying appliance. A satisfactory hardening of the grains can be obtained by the use of less than 5 per cent. of the volatile medium on the dry weight of the finished explosive.

Although we prefer to use non-volatile gelatinizing agents that are sufficiently soluble in the selected volatile organic medium at ordinary temperatures, nevertheless we do not limit our invention to these substances but we include such of these agents as become sufficiently soluble at suitably elevated temperatures. By "sufficiently soluble" we mean that sufficient can be dissolved in the volatile solvent to produce a solution 95 capable of giving the desired hardening effect. This solubility we consider should be not less than 10%. The temperature should not be higher than that at which the powder may be treated with safety but should be high enough to give the necessary solution of the gelatinizer and the desired degree of hardening. We may revolve the wet or dry grains in a heated vessel and spray on to these grains solutions of non-volatile 100 gelatinizing agents at temperatures as high as explosives may be operated upon. The temperature at which the spraying takes place has in some instances a beneficial effect on the hardening operation. The concentration of the gelatinizer in its solvent, the amount of water present in the grains and the temperature at which the operation takes place are all factors governing the degree of hardening effected in our hardening 105 operation.

The non-volatile gelatinizing agents that are suitable for our purpose are:—

- (1) Nitrohydrocarbons.
- (2) Urethanes or esters of carbaminic 110 acids.
- (3) Substituted ureas.
- (4) Condensation products of glycerols and other polyhydric alcohols with aldehydes.
- (5) Homologues of oxanilic ester.
- (6) Non-volatile esters of organic acids.
- (7) Anilids or their homologues, or mixtures thereof.

Each group and each individual member 130

thereof will produce a specific hardening effect depending on its nature and on the proportion of material present as well as the conditions mentioned above, so by choosing 5 mixtures a wide range in degree of hardening may be secured. Examples of some of these gelatinizers applied to another purpose utilizing their combined gelatinizing effect with nitroglycerin are published in British 10 patent specifications Nos. 4940 and 4941 of 1913.

The volatile organic medium suitable for our purpose is chosen from individual members of the usual volatile organic solvents 15 such as alcohol, methylated spirit, amylalcohol benzol, petrol, ether, etc., or combinations of the same, the choice depending on the nature of the non-volatile gelatinizer employed. The organic solvent or mixture of 20 solvents should be so chosen that such dissolves the non-volatile gelatinizer and produces a solution with the desired hardening properties.

So that this form of our invention may be 25 more fully understood, we will describe one example and method of production. A wet mixture of 76 parts of nitrocellulose, 10 parts of barium nitrate, 2 parts of potassium nitrate and 4 parts of mineral jelly, total 92 30 parts, are mixed and incorporated under an edge-runner. This mixture is rubbed through a sieve 10 meshes to the inch and the sifted material placed in steam heated revolving pans until the grains are correctly 35 formed and contain about 50% of water. The correct sizes of grains are sifted out and dried. The dried grains are placed in a suitable revolving vessel, and while this vessel is being revolved, for every 92 parts dry 40 weight of explosive grain, 8 parts of benzyl formanilid in solution in 5 parts of a mixture of one part of alcohol and two parts of benzene is sprayed onto the grains. These grains are then removed from the vessel and 45 the small amount of volatile medium dried out and a well hardened grain results.

In carrying the invention into effect in another form in which the use of a volatile solvent is avoided, we harden wet or dry 50 granulated fibrous nitrocellulose explosives by bringing these granulated explosives into contact with a liquid non-volatile gelatinizer in a finely divided or atomized form, as by a spray. In this method of manufacture we 55 not only avoid the use of volatile solvents, but also eliminate one of the two drying operations at present necessitated in manufacturing hardened granulated fibrous nitrocellulose explosives by the known processes 60 described above.

In this form of our invention, we select either liquid gelatinizers or mixtures of gelatinizers that are liquid at the temperatures it is convenient to work at. A solid gelatinizer may be used by adding a suitable non-

volatile ingredient or ingredients which would have the effect of lowering its melting point without adversely affecting the properties of the powder. The ingredient or ingredients chosen need not necessarily, although they preferably should, possess gelatinizing properties. A suitable example is phenyl urethane to which has been added an equimolecular proportion of tolyl urethane. We place the wet or dry grains in a revolving vessel and while the grains are being moved about spray on to them the gelatinizing agent by any known convenient atomizing or spraying appliance. A satisfactory 70 hardening of the grains can be obtained by 75 comparatively small amounts of the gelatinizing agent, in some cases by as low as 5% on the dry weight of the finished explosive.

Although we prefer to use non-volatile gelatinizing agents that are liquid at ordinary temperatures, nevertheless we do not limit our invention to these liquids. We may revolve the dry or wet grains in a heated vessel and spray on to these grains liquid non-volatile gelatinizing agents at 80 temperatures as high as explosives may be operated upon. The temperature at which spraying takes place has in some instances a beneficial effect on the hardening operation.

The liquid gelatinizing agents that are 85 suitable for our purpose are quite numerous and the following are given as examples, viz., gelatinizers which are liquids at ordinary temperatures:—The liquid nitrohydrocarbons or liquid mixtures of nitrohydrocarbons, ethyl phthalate, phenyl benzyl urethane, formal glycerol, the liquid mixture of formanilid and form-o-toluidid, etc., 90 gelatinizers liquid at temperatures below 50° C., benzyl formanilid, o-tolyl oxamic ester, 95 an equimolecular mixture of methyl phenyl urea and ethyl phenyl urea, etc. Any non-volatile gelatinizing agent, however, may be used, the essential feature being spraying a 100 liquid or liquefied non-volatile gelatinizing agent on to wet or dry granulated nitrocellulose mixtures at convenient temperatures for 105 the purpose of hardening these grains without the use of volatile media.

So that this form of our invention may be 110 more fully understood we will describe one example and method of production. A wet mixture of 76 parts of nitrocellulose, 10 parts of barium nitrate, 2 parts of potassium nitrate and 4 parts of vaseline, total 92 115 parts, are mixed and incorporated under an edge-runner. This mixture is rubbed through a sieve 10 meshes to the inch and the sifted material placed in a steam heated revolving pan until the grains are correctly 120 formed and contain about 50% of water. The correct sizes of grains are then sifted out and placed in a suitable revolving vessel and while this vessel is being revolved, for every 92 parts dry weight of explosive 125 130

grain 8 parts by weight of phenyl benzyl urethane is sprayed on to the grains. The wet grains are then removed from the vessel and dried and a well hardened powder is 5 produced.

In carrying the invention into effect in a further form also avoiding the use of a volatile solvent, we harden wet or dry granulated fibrous nitrocellulose explosives by mixing 10 them with one or a mixture of solid gelatinizers in a fine state of division and causing the adhering particles to effect the required hardening, preferably under rise of temperature. In this form of our invention we 15 select solid gelatinizers or mixtures thereof which melt or act at a temperature at which explosives may be operated upon. The solid gelatinizing agent is reduced to a fine state of division and mixed with the wet or dry 20 granulated fibrous explosive, preferably when warm. This mixture is then placed in a suitably heated vessel and left therein until the hardening effect has taken place. The solid gelatinizers suitable for our pur- 25 pose should melt or act below say about 70° C. and are quite numerous. The following are quoted as examples, viz., methyl acetanilid, formanilid, an equimolecular mixture of methyl phenyl urea and ethyl 30 phenyl urea, benzyl formanilid, phenyl urethane, tolyl urethane and mixtures of these.

So that this form of our invention may be more fully understood we will describe 35 one example and method of production. The same weight of grains of the correct size containing about 50% water and prepared as in the last example, is, while still warm, mixed with 8 parts of finely divided 40 phenyl urethane, and the mixture is placed in a suitably heated revolving vessel. Heat is applied while the vessel is revolving until the mixture has attained the melting point of the gelatinizer or the temperature at 45 which the gelatinizer acts. The wet grains are then removed and dried, and a well hardened powder is produced, in an extremely simple and convenient manner.

In carrying this invention into effect in 50 another form also avoiding the use of volatile organic solvents we harden granulated fibrous nitrocellulose explosives without the use of volatile mediums by spraying on to the dry or nearly dry grains an aqueous so- 55 lution of a non-volatile gelatinizing agent.

We select gelatinizers that are sufficiently soluble in water at the temperatures it is convenient to work at. We place the dry or nearly dry grains in a revolving vessel and 60 while the grains are being moved about bring into contact with them in a finely di- vided or atomized condition an aqueous solu- 65 tion of the gelatinizing agent by means of any convenient atomizing or spraying appli- ance.

Although we prefer to use non-volatile gelatinizing agents that are sufficiently soluble in water at ordinary temperatures, nevertheless we do not limit our invention to these substances, but include such of these 70 agents as become sufficiently soluble at suitably elevated temperatures. We may revolve the dry or nearly dry grains in a heated vessel and spray on to these grains aqueous solutions of non-volatile gelatinizers 75 at temperatures as high as explosives may be operated upon. The temperature at which the spraying takes place has in some instances a beneficial effect on the hardening operation. The concentration of the gelatinizer in the aqueous solution, the amount of moisture present in the grains treated and the temperature at which the operation takes place are all factors of our hardening 80 operation. 85

The non-volatile gelatinizing agents having the requisite characteristics are quite numerous; the following are given only by way of example, viz., formal glycerol, methyl phenyl urea, ethyl phenyl urea, acetanilid, 90 methyl acentanilid, etc. Any water soluble non-volatile gelatinizing agent, however, may be used that is sufficiently soluble in water to harden at the temperatures that are 95 adopted for the operation.

So that this form of our invention may be more fully understood we will describe one example and method of production. A wet mixture of 76 parts of nitrocellulose, 10 parts of barium nitrate, 2 parts of potassium nitrate, total 88 parts, are mixed and incorporated under an edge-runner. This mixture is rubbed through a sieve 10 meshes to the inch and the sifted material placed in a steam heated revolving pan until the 105 grains are correctly formed and contain about 50% of water. The correct sizes of grains are then sifted out and dried until containing less than 5% of water. The dried or nearly dried grains are placed in a suitable 110 revolving vessel and while this vessel is being revolved, for every 88 parts dry weight of explosive grain, 36 parts of an aqueous solution containing 33% methyl phenyl urea is sprayed on to the grains. The wet grains 115 are then removed from the vessel and dried, and a well hardened product results. If desired, the incorporation of a suitable non-volatile gelatinizing agent or agents may be made in the manufacture of the grains, 120 the hardening of the grains being effected thereby.

The term "spray" is employed in the claims to include the application of the gelatinizer or agent in finely subdivided 125 form, whether the agent is liquid or solid at the working temperature: the term "liquid non-volatile gelatinizer" includes such gelatinizers as are liquid at normal temperatures, or become liquefied at or below the 130

working temperature, or are applied in liquid form in aqueous or non-aqueous solution.

Claims:

1. Hardened granulated fibrous nitrocellulose shot-gun explosives in which the hardening has been effected by the aid of non-volatile gelatinizing agents.
2. Processes for producing hardened granulated fibrous nitrocellulose shot-gun explosives which include the step of hardening the particles of the explosive by the aid of non-volatile gelatinizing agents.
3. A method of manufacturing hardened granular fibrous nitrocellulose shot-gun explosives which includes the incorporation of a non-volatile gelatinizing agent in the manufacture of the grains and in bringing about hardening of the grains thereby.
4. A method of manufacturing hardened granular fibrous nitrocellulose shot-gun explosives which includes hardening of the dry or nearly dry grains by the combined gelatinizing effect of a volatile solvent and that of an added non-volatile gelatinizing agent

and subsequently removing the volatile organic medium.

5. Process according to claim 2 wherein the non-volatile gelatinizing agent is applied in the form of a spray.

6. Process according to claim 5 in which the spray is applied to the wet grains.

7. Process according to claim 5 in which a liquid non-volatile gelatinizer is employed.

In testimony whereof we have signed our names to this specification.

WILLIAM RINTOUL.

THOMAS JOSEPH NOLAN.

OLIVER WARD STICKLAND.

Witnesses to the signatures of the above named William Rintoul and Oliver Ward Stickland:

MATTHEW GEORGE JARDINE,  
JOHN DONALD MACKENZIE.

Witnesses to the signature of the above named Thomas Joseph Nolan:

EDWARD FELTON,  
ROBERT EVAN FELTON.